

## UNITED STATES PATENT OFFICE

WILLIAM CURETON, OF CHICAGO, ILLINOIS.

## FOUNDRY SAND.

No Drawing.

Application filed April 6, 1925. Serial No. 21,121.

The invention pertains to the art of molding as practiced in foundries in connection with the production of castings from various kinds of metals, and has particular reference to the composition of the foundry sand from which the molds are made.

In constructing molds for gray iron, malleable iron, and non-ferrous metal castings, the general practice heretofore has been to use a foundry sand which is composed of a mixture of silica sand, some clayey material containing principally alumina, lime, magnesia and iron compounds to give the necessary bonding quality, and some sea coal or other carbon material to give the necessary refractory quality, to all of which a suitable quantity of water is added and thoroughly mixed. The bonding and refractory qualities of this foundry sand are not very high, however, and under some conditions of use it is usual to increase the same, the bonding quality by the addition of flour, pitch compounds, or other organic resinous substances, and the refractory quality by the facing of the molds with graphite, or other high carbon compounds. In constructing molds for steel castings, the practice has been to use a somewhat similar foundry sand which is composed of a purer silica sand, some finely ground fire clay and pitch, and some molasses or other organic resinous compounds mixed with water.

The foundry sands above described have been widely used for years, but such sands have many objectionable characteristics which are reflected disadvantageously in the appearance, surface texture and average cost of the satisfactory castings produced. The sands will stick to the patterns unless moistened with great uniformity, and will pack too hard to allow the gases to escape if too much moisture is used. Furthermore, the sands will fuse in contact with the molten metal, irrespective of the skill with which the sands are prepared, and such fusing or burning of the sands will form gases and slag, will render the surfaces of the castings irregular, and will lower the bonding and refractory qualities of the sands to such an extent as to make a substantial portion of the same unfit for subsequent use.

The object of the present invention is to provide an inexpensive foundry sand which is not open to any of the objections above described.

The foundry sand of the invention con-

sists essentially of a base of silica sand and a binder of a finely ground mineral commercially known as talc, to which mixture is added sufficient water to moisten the same properly. The novel and highly advantageous employment of talc in this association is the salient feature of the invention.

Talc has a lubricating or soapy feeling to the fingers, is soft, and may be easily ground to an impalpable powder having a plastic quality somewhat similar to that found in clays. Talc is chemically known as magnesium silicate,  $H_2Mg_3(SiO_4)_2$ , but one form is an aluminum silicate known as pyrophyllite,  $H_2OAl_2O_3SiO_2$ . While some deposits of the mineral talc cannot be used, probably because of such impurities therein as iron, lime and clayey materials which tend to form gases and slag in the molds, certain deposits found to be sufficiently pure for the purpose have been analyzed with the following results: Silicon 60.2%, magnesia 30.33%, iron oxides and alumina 3.8%, combined water 5.35%, lime 0.9%, and moisture 0.3%.

The silica sand and the talc may be combined in a wide range of proportions, depending of course upon the particular type of casting for which the sand is to be used, the amount of talc being increased as a general rule in proportion to the amount of silica sand as a higher binding quality is required of the sand. One proportioning of the constituent materials of the foundry sand, which has been found to give very good results for one type of casting, is about four parts of silica sand to about one part of talc. It will be understood however that this particular ratio is referred to merely for the purpose of exemplification, and is not to be construed in any way as a restriction of the spirit of the invention to such definite purposes.

Where a very high degree of fineness is desirable in the foundry sand, as is the case in the production of certain types of castings, the sand may contain, in addition to the silica sand and the talc, some ground silica known as silica mesh or flint. The amount of flint used, in proportion to the other constituent materials, depends in large measure upon the fineness of the material.

The foundry sand of the invention is distinctly superior in a number of ways over the sands heretofore used in foundries. The silica sand and the talc, when combined in suitable proportions, form an efficient bond,

The sand is highly refractory, and, where it comes into contact with the molten metal, it will not fuse or be destroyed by the heat of the metal, and only a very small portion 5 of the talc therein will adhere to the casting. The sand may be used repeatedly without material loss in bulk or quality, it being only necessary to add small amounts of talc from time to time to maintain the bonding 10 quality in the sand. Due to the soapy characteristic of the talc in the sand, the patterns may be withdrawn from the molds with ease and will leave a very accurate impression. This advantage is particularly evident when 15 the molds are made with the various types of molding machines now in use. Furthermore, when the molds are rammed hard the sand will still retain its porosity, and excessive moisture will not accumulate in spots, 20 as so often happens in molds made with other kinds of foundry sand. Because of the nature of the sand the moisture may be readily mixed and blended throughout the mass. The foregoing advantages are but a 25 few of those possessed by the foundry sand of the invention, and other advantages will be at once evident to those skilled in the art upon use of the sand.

I claim:

1. A foundry sand composed of a base 30 material and a binder of talc.
2. A foundry sand composed of a base of silica sand and a binder of talc.
3. A foundry sand composed of a relatively large portion of silica sand and a 35 relatively small portion of talc.
4. A foundry sand composed of a base of silica sand and a binder of finely ground talc combined in the approximate proportions of about four parts of silica sand and 40 one part of talc.
5. A foundry sand composed of a base material, talc, and ground silica.
6. A foundry sand composed of silica sand, talc, and flint. 45
7. The method of preparing foundry sand for castings which consists in binding the base material of the sand throughout its mass with talc.
8. The method of preparing foundry sand 50 for castings which consists in binding a base of silica sand throughout its mass with a binder of finely ground talc.

In testimony whereof I have hereunto subscribed my name.

WILLIAM CURETON.